

# UNITED STATES PATENT OFFICE.

CARL LUCKOW, OF COLOGNE-DEUTZ, GERMANY.

## PROCESS OF PRODUCING PEROXID OF LEAD.

SPECIFICATION forming part of Letters Patent No. 626,330, dated June 6, 1899.

Application filed December 31, 1897. Serial No. 665,209. (No specimens.)

*To all whom it may concern:*

Be it known that I, CARL LUCKOW, a subject of the King of Prussia, German Emperor, residing at Cologne-Deutz, Germany, have invented certain new and useful Improvements in Processes of Producing Peroxid of Lead by Means of Electrolysis, of which the following is a specification.

The invention has been patented in England, No. 14,801, dated August 6, 1895.

The object of this invention is to produce peroxid of lead by means of electrolysis.

It consists, essentially, in the use as electrolyte of a salt of sulfuric acid with sodium, potassium, or ammonium in mixture with a salt of chloric acid with sodium, potassium, or ammonium in aqueous solution in connection with anodes of lead. The mixture should be about 99.5 per cent. of one of the salts named above of sulfuric acid and about 0.5 per cent. of one of the salts named above of chloric acid, and the aqueous solution should contain from 0.3 to three per cent. of the mixture, the quantities of salt always calculated free from water. This solution serves as electrolyte. The electrodes are of lead. Under the influence of the electric current the lead of the anode is transformed into peroxid of lead, the hydrogen of the water decomposed by the process escapes, and the oxygen enters into the peroxid of lead. The process goes on continually with the same electrolyte as both

acids remain undecomposed by the action of the current and only the water consumed by the process has to be renewed.

35

Example: A dilute solution one and one-half per cent. strong of a mixture of 99.5 weight parts of sulfate of sodium and 0.5 weight parts of chlorate of sodium forms the electrolyte. Therein the anodes and cathodes are suspended and an electric current passed through. The intensity of this current should be fifty amperes, its density 0.5 amperes pro square decimeter, and its tension about three volts. To facilitate the reaction and to keep the electrolyte in motion, air is carefully blown in during the process.

40 45 50 55

What I claim is—

The herein-described process of producing peroxid of lead by means of electrolysis consisting in using in connection with a lead anode an aqueous solution as electrolyte containing from 0.3 to three per cent. of the sodium, potassium or ammonium salts of sulfuric acid in mixture with the sodium, potassium or ammonium salts of chloric acid, and in passing a current through the said solution, substantially as described.

In witness whereof I have hereunto set my hand in presence of two witnesses.

CARL LUCKOW.

Witnesses:

OTTO STRECKER,  
WILLIAM H. MADDEN.